

1

3,215,520

METHOD OF PRODUCING LUMP ORES  
 Louis George Imperato, Jr., Tenafly, N.J., assignor to  
 Blocked Iron Corporation, a corporation of New York  
 No Drawing. Filed May 27, 1964, Ser. No. 370,674  
 9 Claims. (Cl. 75—3)

This application is a continuation-in-part of my co-pending application Serial No. 34,359, filed June 7, 1960, now abandoned, which was an improvement over the lump ores and methods of producing them disclosed in copending application Serial No. 749,546, filed July 18, 1958, now Patent No. 2,996,372.

This invention relates to lump ores and to methods of producing them and particularly to a lump ore and method of producing such an ore from finely divided materials containing metals in the metallic state, as metallic compounds such as oxides or mixtures thereof. The invention is particularly adapted to the production of lump iron ores from finely divided iron ores, blast furnace flue dust and other sources of iron and iron compounds which are available in a fine state of subdivision.

In the case of iron ore, for example, natural reserves of high grade lump ores are rapidly being depleted by selective mining. It has been increasingly necessary to utilize the more finely divided high grade ores as well as to turn to low grade ores which must be beneficiated. In using such ores it is not uncommon to find them in size ranges such that they pass through a 200 to 325 mesh. In addition to these finely divided natural ores there are large quantities of blast furnace flue dust, fine scale, and similar other sources of iron and iron compounds available in the finely divided state for use in iron and steel-making processes. However, these materials, because of their fineness, tend to fuse and bridge over or to be flushed out with the early slag before accomplishing their metallur-

2

gical function in the open hearth steel-making furnace or to be carried out through the top of the blast furnace in iron making and are not suitable in their naturally occurring condition for use in open-hearth steel-making furnaces or in blast furnaces. In addition, many of these ores are high in sulfur and similar undesirable elements. In order to take advantage of these materials, it has been the practice to take these finely divided materials and either sinter, pelletize or nodulize them by heating to high temperatures or by bonding them together with hydraulic cement. All of these practices are relatively expensive and in some instances are undesirable because of the increased amounts of impurities such as silica and alumina which are introduced into the ore by the bonding practice.

15 I have discovered an improved lump ore product produced from such finely divided materials and a method of producing it. The lump ores produced according to my invention are free from the objections common to the presently used ores produced by sintering, pelletizing and nodulizing finely divided materials. The lump ore of this invention has the desirable thermal and chemical characteristics of natural lump ore, and has the strength and resistance to crushing characteristic of natural lump ores. The lump ore of this invention is, moreover, free from 20 undesirable added impurities, contains bonding materials similar to the fluxing materials normally used in metallurgical practices, may be formed of blended or mixed iron-containing materials and has a built-in sulfur eliminating component.

25 30 Amberg Patent 2,844,457 provides a method of forming lump ore products from finely divided metal containing material by bonding the material together with an alkaline earth carbonate and formed by mixing the finely divided metal containing material with an oxide or hydroxide or calcium, mixed calcium and magnesium in the presence of moisture within specific limits forming the lumps and treating them with carbonic acid gas. This practice pro-

Table I

| Batch    | Materials                                                                                                  | Parts on<br>Dry Wgt.<br>of Ore                 | Exposure to Carbon Dioxide<br>Atmosphere                         |          |           |
|----------|------------------------------------------------------------------------------------------------------------|------------------------------------------------|------------------------------------------------------------------|----------|-----------|
|          |                                                                                                            |                                                | 30 mins.                                                         | 60 mins. | 120 mins. |
| I-----   | Liberian Ore/Conc. (50%/50%)<br>Hydrated Lime<br>Calcium Chloride<br>Molasses<br>Sodium Hydroxide<br>Water | 100.00<br>4.00<br>0.20<br>0.40<br>0.27<br>6.00 | 82%                                                              | 89%      | 91%       |
|          |                                                                                                            |                                                | (Retained on 0.371 mesh sieve after 50 rev. on A.S.T.M. tumbler) |          |           |
| II-----  | Liberian Ore/Conc. (50%/50%)<br>Hydrated Lime<br>Molasses<br>Sodium Hydroxide<br>Water                     | 100.00<br>4.00<br>0.40<br>0.27<br>6.50         | 75%                                                              | 83%      | 83%       |
|          |                                                                                                            |                                                | (Retained on 0.371 mesh sieve after 50 rev. on A.S.T.M. tumbler) |          |           |
| III----- | Liberian Ore/Conc. (50%/50%)<br>Hydrated Lime<br>Calcium Chloride<br>Molasses<br>Water                     | 100.00<br>4.00<br>0.20<br>0.40<br>6.50         | 61%                                                              | 69%      | 71%       |
|          |                                                                                                            |                                                | (Retained on 0.371 mesh sieve after 50 rev. on A.S.T.M. tumbler) |          |           |
| IV-----  | Liberian Ore/Conc. (50%/50%)<br>Hydrated Lime<br>Calcium Chloride<br>Water                                 | 100.00<br>4.00<br>0.20<br>7.00                 | 38%                                                              | 42%      | 46%       |
|          |                                                                                                            |                                                | (Retained on 0.371 mesh sieve after 50 rev. on A.S.T.M. tumbler) |          |           |
| V-----   | Liberian Ore/Conc. (50%/50%)<br>Hydrated Lime<br>Water                                                     | 100.00<br>4.00<br>7.25                         | 29%                                                              | 30%      | 34%       |
|          |                                                                                                            |                                                | (Retained on 0.371 mesh sieve after 50 rev. on A.S.T.M. tumbler) |          |           |
| VI-----  | Liberian Ore/Conc. (50%/50%)<br>Hydrated Lime<br>Sodium Hydroxide<br>Water                                 | 100.00<br>4.00<br>0.27<br>7.00                 | 29%                                                              | 29%      | 26%       |
|          |                                                                                                            |                                                | (Retained on 0.371 mesh sieve after 50 rev. on A.S.T.M. tumbler) |          |           |
| VII----- | Liberian Ore/Conc. (50%/50%)<br>Hydrated Lime<br>Calcium Chloride<br>Sodium Hydroxide<br>Water             | 100.00<br>4.00<br>0.20<br>0.27<br>7.00         | 20%                                                              | 15%      | 22%       |
|          |                                                                                                            |                                                | (Retained on 0.371 mesh sieve after 50 rev. on A.S.T.M. tumbler) |          |           |

duces a lump ore product having highly desirable characteristics and being superior to anything previously available. I have found, however, that the product of the Amberg patent can be significantly improved particularly when finely divided high calcium oxides or hydroxides are used in the mixture, and when the ore contains significant amounts of sulfur. I have discovered that the addition of sugars, such as maltose, sucrose, dextrose and glucose, and sugar containing materials, such as molasses, syrups and carbohydrates and other materials such as starch and the sodium salt of ethylene-diamene tetraacetic acid as disclosed in Patent No. 2,996,372 which are capable of solubilizing alkaline earth metals to the mixture, together with certain basic compounds of the alkali metals prior to carbonation will significantly improve the resistance of the lump ores to crushing and disintegration under impact,

10

5

the following examples which show the significance of the practice according to my invention:

#### EXAMPLE I

A Liberian ore concentrate was divided into seven parts and formed into various admixtures. These mixtures were exposed to carbon dioxide for varying times and the block strength determined as percent remaining on .371 mesh sieve after 50 revolutions in an A.S.T.M. tumbler. The results appear in Table I above.

#### EXAMPLE II

Venezuelan ore fines were divided into two portions. These portions were mixed and formed as indicated in Table II below. These mixtures were briquetted and treated with carbon dioxide for 2½ hours. After carbonation, the briquettes were tumbled as in Example I. The results are shown in Table II.

Table II

| Batch | Materials                                                                                              | Parts on<br>Dry Wgt.<br>of Ore                  | Exposure to Carbon Dioxide<br>Atmosphere (in minutes)                      |          |           |
|-------|--------------------------------------------------------------------------------------------------------|-------------------------------------------------|----------------------------------------------------------------------------|----------|-----------|
|       |                                                                                                        |                                                 | 30 mins.                                                                   | 60 mins. | 180 mins. |
| I     | —¾" Venezuelan Ore Fines<br>Hydrated Lime<br>Calcium Chloride<br>Molasses<br>Sodium Hydroxide<br>Water | 100.00<br>5.00<br>0.20<br>0.50<br>0.27<br>12.00 | 91%<br>(Retained on 0.371 mesh sieve after<br>50 rev. on A.S.T.M. tumbler) | 92%      | —         |
| II    | —¾" Venezuelan Ore Fines<br>Hydrated Lime<br>Calcium Chloride<br>Molasses<br>Water                     | 100.00<br>5.00<br>0.20<br>0.50<br>12.00         | 68%<br>(Retained on 0.371 mesh sieve after<br>50 rev. on A.S.T.M. tumbler) | 66%      | 82%       |

as well as providing the power to eliminate sulfur from the bath. I have found that the addition of small amounts of sugars and certain solubilizing agents for calcium and magnesium oxides and hydroxides, particularly in the range .025 to 1% by weight together with such basic alkali metal compounds will more than double the resistance of the lump ores to physical shock. By alkali metals I mean

45

50

the same Venezuelan ore used in Example II was admixed with varying percentages of sodium hydroxide, and with hydrated lime, molasses, calcium chloride, and water, as shown in Table III below. The mixture was briquetted, and treated with carbon dioxide for 60 minutes. The resulting briquettes were tumbled and tested as in Example I with the following results.

Table III

| Batch        | Materials                                                                          | Parts on<br>Dry Wgt.<br>of Ore          | Exposure<br>to Carbon<br>Dioxide,<br>mins. | Percent of Sodium Hydroxide Added |      |      |      |      |      |
|--------------|------------------------------------------------------------------------------------|-----------------------------------------|--------------------------------------------|-----------------------------------|------|------|------|------|------|
|              |                                                                                    |                                         |                                            | 0.00                              | 0.14 | 0.27 | 0.41 | 0.54 | 0.78 |
| I through IV | —¾" Venezuelan Ore Fines<br>Hydrated Lime<br>Molasses<br>Calcium Chloride<br>Water | 100.00<br>5.00<br>0.50<br>0.20<br>12.00 | 60                                         | 66%                               | 76%  | 92%  | 85%  | 85%  | 85%  |

#### EXAMPLE IV

amines). These alkali metal oxides and hydroxides are added in an amount equal to at least 0.1% by weight and preferably between about 0.15 to 0.35% by weight. The invention can perhaps best be explained by reference to

75

The identical process of Example III was carried out substituting varied percentages of potassium hydroxide for the varied percentages of sodium hydroxide of Ex-

ample III. The pieces were tested with the following results.

The industry accepted standard is 5 to 10 drops to failure.

Table IV

| Batch        | Materials                                                        | Parts on<br>Wgt. of<br>Dry Ore | Exposure<br>to Carbon<br>Dioxide,<br>mins. | Percent of Potassium<br>Hydroxide Added |      |      |
|--------------|------------------------------------------------------------------|--------------------------------|--------------------------------------------|-----------------------------------------|------|------|
|              |                                                                  |                                |                                            | 0.00                                    | 0.14 | 0.27 |
| I through IV | - $\frac{3}{4}$ " Venezuelan Ore Fines                           | 100.00                         | 90                                         | 66%                                     | 85%  | 91%  |
|              | Hydrated Lime                                                    | 5.00                           |                                            |                                         |      |      |
|              | Molasses                                                         | 0.50                           |                                            |                                         |      |      |
|              | Calcium Chloride                                                 | 0.20                           |                                            |                                         |      |      |
|              | Water                                                            | 12.00                          |                                            |                                         |      |      |
|              | (Retained on 0.371 mesh sieve after 50 rev. on A.S.T.M. tumbler) |                                |                                            |                                         |      |      |

## EXAMPLE V

A specular hematite ore was admixed in the proportions shown in Table V. The mixture was briquetted and treated with carbon dioxide for 2 hrs. The resulting blocks were tested by tumbling as described in Example I with the following results.

20

## EXAMPLE VII

In order to compare the efficiency of other basic compounds of alkali metals and ammonium, magnetite concentrates were admixed in the proportions shown in Table VII. These mixtures were briquetted and subjected to

Table V

| Batch          | Materials                 | Parts on<br>Dry Wgt.<br>of Ore | Strength Index Percent<br>Retained on a 0.371 Mesh<br>Sieve after 50 Revolutions<br>in an A.S.T.M. Tumbler |
|----------------|---------------------------|--------------------------------|------------------------------------------------------------------------------------------------------------|
| I through VI   | Lac Jeannine Concentrates | 100.00                         | 82                                                                                                         |
|                | Hydrated Lime             | 5.00                           |                                                                                                            |
|                | Calcium Chloride          | 0.20                           |                                                                                                            |
|                | Molasses                  | 0.50                           |                                                                                                            |
|                | Water                     | 4.82                           |                                                                                                            |
| VII through IX | Lac Jeannine Concentrates | 100.00                         | 22                                                                                                         |
|                | Hydrated Lime             | 5.00                           |                                                                                                            |
|                | Calcium Chloride          | 0.20                           |                                                                                                            |
|                | Sodium Hydroxide          | 0.27                           |                                                                                                            |
|                | Water                     | 3.95                           |                                                                                                            |
| X through XVII | Lac Jeannine Concentrates | 100.00                         | 90                                                                                                         |
|                | Hydrated Lime             | 5.00                           |                                                                                                            |
|                | Calcium Chloride          | 0.20                           |                                                                                                            |
|                | Molasses                  | 0.50                           |                                                                                                            |
|                | Sodium Hydroxide          | 0.27                           |                                                                                                            |
|                | Water                     | 3.95                           |                                                                                                            |

## EXAMPLE VI

In order to determine the effect of various additives on green strength Venezuelan ore fines were admixed in the proportions shown in Table VI below. These mixtures were formed into  $\frac{1}{2}$  inch pellets and dropped from a height of 12" to a steel plate and the number of drops to fracture recorded as a 20 ball average.

50 a treatment with carbon-dioxide for 2 hours. The resulting briquettes were tested in the manner outlined in Example I with the following results. In the table "Mea" is monoethanol amine and the semicolons separating the percentages indicate percentages obtained on separate determinations.

55

Table VI

| Batch  | Materials                              | Parts on<br>Dry Wgt.<br>of Ore | Percent of<br>Moisture of<br>Formed Pel-<br>let | Strength<br>Index Aver-<br>age Drops<br>to Failure |
|--------|----------------------------------------|--------------------------------|-------------------------------------------------|----------------------------------------------------|
| I      | - $\frac{1}{2}$ " Venezuelan Ore Fines | 100.00                         |                                                 |                                                    |
|        | Hydrated Lime                          | 5.00                           | 11.62                                           | 20                                                 |
|        | Calcium Chloride                       | 0.20                           |                                                 |                                                    |
|        | Water                                  | 12.00                          |                                                 |                                                    |
| II+III | - $\frac{1}{2}$ " Venezuelan Ore Fines | 100.00                         | 10.8                                            | 35.34                                              |
|        | Hydrated Lime                          | 5.00                           |                                                 |                                                    |
|        | Calcium Chloride                       | 0.20                           |                                                 |                                                    |
|        | Molasses                               | 0.50                           |                                                 |                                                    |
|        | Water                                  | 11.00                          |                                                 |                                                    |
| IV+V   | - $\frac{1}{2}$ " Venezuelan Ore Fines | 100.00                         | 10.5                                            | 37.32                                              |
|        | Hydrated Lime                          | 5.00                           |                                                 |                                                    |
|        | Calcium Chloride                       | 0.20                           |                                                 |                                                    |
|        | Molasses                               | 0.50                           |                                                 |                                                    |
|        | Sodium Hydroxide                       | 0.27                           |                                                 |                                                    |
|        | Water                                  | 10.00                          |                                                 |                                                    |

Table VII

| Batch | Materials                                                                                                                                         | Parts on Dry Wgt.<br>of Ore                    | Tumbler Test: Percent<br>Retained on a 0.371 Mesh<br>Sieve After 200 Revolu-<br>tions in an A.S.T.M.<br>Tumbler |
|-------|---------------------------------------------------------------------------------------------------------------------------------------------------|------------------------------------------------|-----------------------------------------------------------------------------------------------------------------|
| I     | Magnetite Concentrates.....<br>Hydrated Lime.....<br>CaCl <sub>2</sub> .....<br>H <sub>2</sub> O.....                                             | 100.00<br>5.00<br>0.20<br>5.93                 | 59; 56%                                                                                                         |
| II    | Magnetite Concentrates.....<br>Hydrated Lime.....<br>CaCl <sub>2</sub> .....<br>Molasses.....<br>H <sub>2</sub> O.....                            | 100.00<br>5.00<br>0.20<br>0.50<br>5.49         | 68; 65%                                                                                                         |
| III   | Magnetite Concentrates.....<br>Hydrated Lime.....<br>CaCl <sub>2</sub> .....<br>Molasses.....<br>Mea.....<br>H <sub>2</sub> O.....                | 100.00<br>5.00<br>0.20<br>0.50<br>0.25<br>5.38 | 79; 77%                                                                                                         |
| IV    | Magnetite Concentrates.....<br>Hydrated Lime.....<br>CaCl <sub>2</sub> .....<br>Molasses.....<br>Ammonium Hydroxide.....<br>H <sub>2</sub> O..... | 100.00<br>5.00<br>0.20<br>0.50<br>0.25<br>5.16 | 75%                                                                                                             |
| V     | Magnetite Concentrates.....<br>Hydrated Lime.....<br>CaCl <sub>2</sub> .....<br>Molasses.....<br>Sodium Hydroxide.....<br>H <sub>2</sub> O.....   | 100.00<br>5.00<br>0.20<br>0.50<br>0.20<br>4.93 | 73%                                                                                                             |
| VI    | Magnetite Concentrates.....<br>Hydrated Lime.....<br>CaCl <sub>2</sub> .....<br>Molasses.....<br>Potassium Sulfate.....<br>H <sub>2</sub> O.....  | 100.00<br>5.00<br>0.20<br>0.50<br>0.75<br>5.16 | 71%                                                                                                             |

The combination of an alkaline earth solubilizing agent such as molasses with a basic compound of an alkali metal or ammonium, a hydroxide of calcium or magnesium and an ore appears to have a profound synergistic effect in producing high green strength and high cured 40 strength. Both of these properties are of great importance in the industry. Moreover, a lesser amount of water in the forming process is needed and, therefore, less drying prior to carbonation. In addition, the alkali metal compounds appear to have some favorable desulfurizing action since they are fixed in the mixture adjacent to the ore and are immediately available to react as the ore is melted.

In the foregoing specification, I have set out certain preferred practices and embodiments of my invention, however, it will be understood that the invention may be otherwise practiced within the scope of the following claims.

I claim:

1. The method of producing lump ore from finely divided iron containing materials, comprising the steps of admixing the finely divided material with at least one of the group consisting of the oxides and hydroxides of alkaline earth metals and with a material capable of solubilizing alkaline earth metals selected from the group consisting of water soluble carbohydrates and the sodium salt of ethylene-diamene tetraacetic acid, and at least 0.1% of an alkaline compound selected from the group consisting of alkali metal oxides and hydroxides, ammonium compounds and amines, forming the mixture into lumps and reacting the resulting lumps with carbon dioxide in the presence of moisture to form alkaline earth oxide in the presence of moisture to form alkaline earth carbonates prior to charging in a metallurgical furnace.

2. The method of producing lump ore from finely divided iron-containing materials, comprising the steps of admixing the finely divided material with at least one of the group consisting of the oxides and hydroxides of alkaline earth metals and mixtures thereof, with a sugar containing material, and at least 0.1% of an alkaline compound selected from the group consisting of alkali

metal oxides and hydroxides, ammonium compounds and amines, forming the mixture into lumps, and reacting the resulting lumps with carbon dioxide in the presence of moisture to form alkaline earth carbonates prior to charging in a metallurgical furnace.

3. The method of producing lump ore from finely divided iron-containing materials, comprising the steps of admixing the finely divided material with at least one of the group consisting of the oxides and hydroxides of alkaline earth metals and a material capable of solubilizing alkaline earth metals selected from the group consisting of water soluble carbohydrates and the sodium salt of ethylene-diamene tetraacetic acid, and at least 0.1% of an alkaline compound selected from the group consisting of alkali metal oxides and hydroxides, ammonium compounds and amines, forming the mixture into lumps and reacting the resulting mixture with carbon dioxide in the presence of up to about 10% moisture and at least one soluble salt from the group consisting of the chlorides, sulfates and carbonates of alkali metals, alkaline earth metals and iron to form alkaline earth carbonates prior to charging in a metallurgical furnace.

4. The method of producing lump iron ore from finely divided iron-containing materials, comprising the steps of admixing the finely divided material with at least one of the oxides and hydroxides of calcium together with at least one starch containing material, and at least 0.1% of an alkali metal hydroxide and reacting the resulting mixture with carbon dioxide in the presence of up to about 10% moisture prior to charging in a metallurgical furnace whereby to form calcium carbonate in the formed lumps.

5. The method of producing lump iron ore from finely divided iron-containing materials, comprising the steps of admixing the finely divided material with at least one of the oxides and hydroxides of calcium, glucose, and with at least 0.1% of an alkali metal hydroxide in the presence of moisture, forming the resulting mixture into lumps and reacting the formed lumps prior to charging in a metallurgical furnace with carbonic acid gas in the

presence of up to about 10% moisture to cause crystallization of calcium carbonate in the interstices of the formed lumps.

6. The method of producing lump iron ore from finely divided iron-containing materials, comprising the steps of admixing the finely divided material with at least one of the oxides and hydroxides of calcium, maltose, and with at least 0.1% of an alkali metal hydroxide in the presence of moisture, forming the resulting mixture into lumps and reacting the formed lumps prior to charging in a metallurgical furnace with carbonic acid gas in the presence of up to about 10% moisture to cause crystallization of calcium carbonate in the interstices of the formed lumps.

7. The method of producing lump iron ore from finely divided iron-containing materials, comprising the steps of admixing the finely divided material with at least one of the oxides and hydroxides of calcium, dextrose, and with at least 0.1% of an alkali metal hydroxide in the presence of moisture, forming the resulting mixture into lumps and reacting the formed lumps prior to charging in a metallurgical furnace with carbonic acid gas in the presence of up to about 10% moisture to cause crystallization of calcium carbonate in the interstices of the formed lumps.

8. The method of producing lump iron ore from finely divided iron-containing materials, comprising the steps of admixing the finely divided material with at least one of the oxides and hydroxides of calcium, fructose, and with at least 0.1% of an alkali metal hydroxide in the presence of moisture, forming the resulting mixture into

lumps and reacting the formed lumps prior to charging in a metallurgical furnace with carbonic acid gas in the presence of up to about 10% moisture to cause crystallization of calcium carbonate in the interstices of the formed lumps.

9. The method of producing lump iron ore from finely divided iron-containing materials, comprising the steps of admixing the finely ground material with at least one of the group consisting of the alkaline earth metal oxides and hydroxides in an amount equivalent to about 2% to 8% of oxide based on the dry weight of the ore, from about 0.025% to 2% by weight of a stabilizing agent for alkaline earth metals selected from the group consisting of water soluble carbohydrates and the sodium salt of ethylene-diamine tetraacetic acid, and about 0.1 to 0.5% of a material selected from the group consisting of alkali metal oxides and hydroxides, amines and ammonium hydroxide, forming the resulting mixture into lumps in the presence of up to about 10% moisture, and reacting the formed lumps with carbon dioxide to convert at least a part of the admixed member of the group oxide and hydroxide to carbonate, prior to charging in a metallurgical furnace.

25

#### References Cited by the Examiner

##### UNITED STATES PATENTS

|           |       |          |       |      |
|-----------|-------|----------|-------|------|
| 2,914,394 | 11/59 | Dohmen   | ----- | 75—3 |
| 2,931,717 | 4/60  | Lee      | ----- | 75—3 |
| 2,996,372 | 8/61  | Imperato | ----- | 75—3 |

BENJAMIN HENKIN, Primary Examiner.